

## UNITED STATES PATENT OFFICE

2,482,917

## SCROOPING COMPOSITION

Saul Kaplan, Teaneck, N. J., assignor to Onyx Oil  
& Chemical Company, Jersey City, N. J., a corporation of Delaware

No Drawing. Application May 16, 1947,  
Serial No. 748,663

3 Claims. (Cl. 106—135)

1

This invention relates to improvements in the art of imparting scroop to fabrics, and more particularly to new compositions which are useful for that purpose. Of particular importance is the application of the invention to knitted rayon, although yarn or other fabrics or textiles may be treated in accordance with the invention. This application represents a continuation in part of my application, Serial No. 453,416, filed August 3, 1942, now abandoned.

Scroop is a characteristic feel or texture of fabrics perhaps best characterized as the crisp rustle of silk and other fabrics. It is common to treat many fabrics, particularly rayon and silk, to impart or increase their scroop. For this purpose silk is treated with soap and then with acid to liberate fatty acids on the fibers. Weak organic acids, such as formic, acetic, lactic, or tartaric acids are sometimes used alone, particularly with silk, as these products are not ordinarily sufficiently effective with rayon. Emulsions of the higher fatty alcohols, such as oleyl alcohol, are used for imparting scroop to fabrics, particularly rayon.

In accordance with the present invention, emulsions of butoxyethyl stearate are used to impart scroop to textiles, and particularly knitted rayon. These emulsions are of the oil-in-water type, with the disperse phase comprising butoxyethyl stearate and the continuous phase is an aqueous medium containing a film-forming protective colloid, such as a gum, gelatin, or the like. In addition to these necessary constituents, the emulsions may contain other material such as emulsifying agents, preservatives, and weakly acidic material, such as a weak organic acid or an acid salt of an organic acid or an acid salt of an inorganic acid, such as aluminum sulfate.

The use of emulsifying agents is ordinarily desirable to reduce the time and power required to produce a stable emulsion; but care must be taken that the emulsifying agent used is compatible with the other constituents of the emulsions and other materials in conjunction with which the emulsions may be used. Many emulsifying agents exert a decided softening effect which radically reduces the scrooping effect if used in any substantial quantity; but ordinarily effective emulsions can be obtained with the use of quantities of emulsifying agent too small to have this deleterious result.

Preservatives in some instances are required because of the protective colloids used. Thus if gum arabic or gelatin or some similar material is used as the film-forming protective colloid, it is ordinarily desirable to use a preservative.

The acid materials to which reference has been made ordinarily increase the effectiveness of the other constituents in imparting scroop to the textile. Some of them have a preservative action

2

and so permit a decrease in the amount of preservative required. Acid materials are also desirable because they neutralize any alkaline materials left on the textile in processing prior to the scrooping treatment.

Advantageously the disperse phase consists only of butoxyethyl stearate, together with a small amount of an emulsifying agent if an oil-soluble emulsifying agent is used. However, the butoxyethyl may be extended by means of a mineral oil, such as one of a viscosity of 50 to 100 seconds Saybolt, at 100° F. Such a mineral oil may be used in quantities up to 50 or 60% without reducing the scrooping effect too radically. Relatively small quantities of waxes may also be included in the disperse phase, but if waxes are used in quantities over about 10%, the scroop is decreased and emulsification difficulties may be encountered with some protective colloids.

20 The continuous phase consists of an aqueous solution of a film-forming protective colloid. Among the colloids which may be used are gelatin (as gelatin or glue), gum arabic, gum ghatti, casein, methyl cellulose, gum tragacanth, gum karaya, gum shiraz, starch, soluble alginates, polyvinyl alcohol, locust bean gum, casein-aluminum formate complex, and the like.

25 Among the acidic materials which may be included in the continuous phase, if the acidic material is used, are the weak organic acids, such as formic, acetic, lactic, glycolic, citric, tartaric, phthalic, maleic, succinic, and malic acid; acidic salts of organic acids, such as aluminum formate or acetate, (both normal and basic salts), ammonium lactate, ammonium oxalate, zinc acetate and zinc formate; and acidic salts of inorganic acids, such as aluminum sulfate, zinc sulfate, ammonium sulfamate, aluminum sulfamate, zinc sulfamate, mon ammonium phosphate, and di ammonium phosphate.

30 Both oil-soluble and water-soluble emulsifying agents may be used, including the petroleum sulfonates, mahogany soaps, fatty alcohol sulfates, salts of alkylated naphthalene sulfonates, sulfo carboxylic esters (such as dioctyl sodium sulfo succinate), acylated protein degradation products, higher alcohol secondary sulfates, alkyl sulfonates, such as sodium cetyl sulfonate, sulfated oils, condensates of alkylene oxides and fatty acids or fatty alcohols, soaps, such as triethanolamine oleate, as well as the various cation active wetting agents, such as the quaternary ammonium compounds, pyridinium compounds, oxazolodinium compounds, etc. Only small amounts of the emulsifying agents may be used, as most of them exert a softening effect detrimental to the scroop, particularly the sulfonated oils and cation active materials.

35 40 45 50 55 60 The invention will be further illustrated by

the following examples, but it is not limited thereto.

*Example 1.*—A scooping composition is prepared from the following:

|                                           | Pounds |
|-------------------------------------------|--------|
| Butyl "Cellosolve" stearate               | 20.0   |
| Gelatin                                   | 2.0    |
| Sodium di-isopropyl naphthalene sulfonate | 0.1    |
| Sodium pentachlor phenate                 | 0.2    |
| Water                                     | 77.7   |

The gelatin is soaked in part of the water, and the mixture is heated to dissolve it. The sodium di-isopropyl naphthalene sulfonate is dissolved in 2 parts of the water, and added to the gelatin. The butyl "Cellosolve" stearate, at a temperature of from 40 to 50° C. is then added to this mixture while it is agitated rapidly, such as with a turbo mixer. The balance of the water and preservative is then added. The mixture may then, if desired, be passed through a colloid mill or homogenizer. A stable emulsion results, and if creaming occurs on prolonged storage, agitation will restore its homogeneity, and its usefulness is unimpaired.

*Example 2.*—A scooping composition is prepared from the following:

|                                            | Pounds |
|--------------------------------------------|--------|
| Butyl "Cellosolve" stearate                | 15     |
| Gum arabic solution 50% suitably preserved | 6      |
| Water                                      | 79     |

The materials are mixed and suitably emulsified. If 10 to 15 pounds of gum arabic solution are used, the emulsification is easier.

*Example 3.*—A scooping composition is prepared from the following:

|                                 | Pounds |
|---------------------------------|--------|
| Butyl "Cellosolve" stearate     | 16     |
| Casein-aluminum formate complex | 50     |
| Water                           | 34     |

The butyl "Cellosolve" stearate is emulsified in the casein-aluminum formate complex at the temperature of liquefaction of the complex, and then the water is added.

*Example 4.*—A skein of cuprammonium yarn, previously freed from oil and size by a conventional boil-off, and which may have subsequently been dyed, is worked in a bath containing 1 to 5% of any of the compositions of the previous examples. The percentage is based on the weight of the skein, and the amount of the water used may be from 10 to 25 times the weight of the skein. After 15 minutes, the skein is extracted, and dried. It possesses a firm crunchy feel. The effect is somewhat enhanced if from 0.5% to 2% of formic acid is added to the bath a few minutes before the emulsion is introduced.

*Example 5.*—Rayon knit goods, suitably scoured, and dyed, if desired, is impregnated with a 2% solution of any of the emulsions of the foregoing examples in a suitable apparatus, such as a mangle. Upon drying, the goods have a good scoop, and in the case of some constructions, which are brushed to produce a nap, still retain the scoop, despite the mechanical working.

*Example 6.*—Rayon knit goods are dyed, after scouring, in a reel type machine, and the dye bath is dropped. The machine is filled with water at about 100° F., and 2% of an emulsion of any of the previous examples (based on the weight of the goods) is added. After running 15 minutes, the liquor is dropped, the goods extracted, and dried. The effect may be increased by adding,

with the emulsion, about 0.5% of maleic acid, based on the weight of the goods.

Naturally some of the emulsions illustrated above are more efficient than others, and some tend to produce a more lasting scoop than others. In general, an increase in the quantity of butoxy ethyl stearate in an emulsion increases its effectiveness, those containing amounts of butoxy ethyl stearate ranging up to 40% generally giving a better and more lasting scoop than those containing 10% or less, if used at the same concentration.

In formulating any emulsion to be used in imparting scoop to a fabric, care must be taken that the various constituents are compatible and also that they are compatible with other materials in conjunction with which they are to be used. Thus, if the film-forming protective colloid used is gum arabic, aluminum acetate should not be included in the emulsion as its use will lead to precipitation when the emulsion is diluted, if not before. Similarly, where the emulsions are to be used in conjunction with other finishes, such as water repellents, fire proofing compounds, and weighting compositions, ingredients which are incompatible with these other finishes should not be included in the emulsions.

When an emulsifying agent is used in preparing the emulsion, it is usually best to make a practical test of the emulsion to determine what proportion of the emulsifying agent can be used without appreciably affecting the scoop. Most emulsifying agents will serve their purpose effectively in quantities below those which produce a noticeable effect upon the scoop obtained with the final product, but nevertheless it is ordinarily advisable to test the material before using it.

I claim:

1. A scooping composition in the form of an oil-in-water emulsion comprising a continuous phase of an aqueous solution of a film-forming organic colloid and a dispersed phase including butoxyethyl stearate, the butoxyethyl stearate being present in an amount effective to impart scoop to rayon and silk when treated with the composition.

2. A scooping composition in the form of an oil-in-water emulsion comprising a continuous phase of an aqueous solution of an aluminum formate-casein complex and a dispersed phase including butoxyethyl stearate, the butoxyethyl stearate being present in an amount effective to impart scoop to rayon and silk when treated with the composition.

3. A scooping composition in the form of an oil-in-water emulsion comprising a continuous phase of an aqueous solution of gelatin and sodium di-isopropyl naphthalene sulfonate and a dispersed phase including butoxyethyl stearate, the butoxyethyl stearate being present in an amount effective to impart scoop to rayon and silk when treated with the composition.

SAUL KAPLAN.

#### REFERENCES CITED

The following references are of record in the file of this patent:

#### UNITED STATES PATENTS

| 70 | Number    | Name           | Date          |
|----|-----------|----------------|---------------|
|    | 2,015,865 | Muller         | Oct. 1, 1935  |
|    | 2,069,303 | Dreyfus et al. | Feb. 2, 1937  |
|    | 2,176,402 | Koch           | Oct. 17, 1939 |
|    | 2,190,331 | Mosher         | Feb. 13, 1940 |
| 75 | 2,221,674 | Ellis          | Nov. 12, 1940 |

**Certificate of Correction**

Patent No. 2,482,917

September 27, 1949

**SAUL KAPLAN**

It is hereby certified that error appears in the printed specification of the above numbered patent requiring correction as follows:

Column 2, lines 9 and 10, after the word "butoxyethyl" insert *stearate*;  
and that the said Letters Patent should be read with this correction therein that the same may conform to the record of the case in the Patent Office.

Signed and sealed this 31st day of January, A. D. 1950.

[~~SEAL~~]

**THOMAS F. MURPHY,**  
*Assistant Commissioner of Patents.*